

[54] **METHOD FOR PROCESSING CELLULOSE CONTAINING MATERIALS TO IMPART THERETO FLAME RESISTANCE**[75] Inventor: **Kosuke Yamamoto**, Kamakura, Japan[73] Assignee: **Mitsui Toatsu Chemicals, Incorporated**, Tokyo, Japan[22] Filed: **Feb. 28, 1974**[21] Appl. No.: **446,802**[30] **Foreign Application Priority Data**

Feb. 28, 1973 Japan ..... 48-23266

[52] U.S. Cl. .... **427/396**; 106/15 FP; 252/8.1; 260/932; 260/DIG. 24; 427/354; 427/382; 428/276; 428/921[51] Int. Cl. .... **C09D 5/18**

[58] Field of Search ..... 117/143 R, 136, 137, 147,

117/154, 118; 8/116 P; 252/8.1; 260/932; 106/15 FP; 427/354, 382, 396; 428/276, 921

## [56]

**References Cited**

## UNITED STATES PATENTS

|           |         |                    |           |
|-----------|---------|--------------------|-----------|
| 3,658,952 | 4/1972  | Nachbur et al..... | 117/137 X |
| 3,699,192 | 10/1972 | Moretti.....       | 117/136 X |
| 3,754,981 | 8/1973  | Nachbur et al..... | 117/136   |
| 3,763,283 | 10/1973 | Curgan .....       | 117/136 X |

Primary Examiner—Michael R. Lusignan  
Attorney, Agent, or Firm—Lane, Aitken, Dunner & Ziems

## [57]

**ABSTRACT**

This invention relates to a new method for treating cellulosic materials to imparting flame resistance coupled with excellent fastness or resistance to washing and crease resistance. The process employs a phosphorus compound containing methylene ether bonds and a residue of a nitrogen containing compound capable of forming a dimethylol compound.

**4 Claims, No Drawings**

**METHOD FOR PROCESSING CELLULOSE  
CONTAINING MATERIALS TO IMPART THERETO  
FLAME RESISTANCE**

**BACKGROUND OF THE INVENTION**

For imparting flame resistance to cellulose containing fibrous materials, the urea phosphate process is conventionally employed (see, for example, Japanese Patent Publication No. 4950/1962). The cloth processed by the urea phosphate process suffers from many defects, for example, poor resistance to washing, a rough finish and a poor feel as well as a great reduction in strength.

A relatively new method for flameproofing is disclosed in Japanese Pat. No. 691,726. This patent, teaches that N-methylolated phosphorus compounds bearing a methylene ether bond and obtained by condensation of 3-dimethylphosphonopropionic acid methylolamide, followed by methylolation with a reagent capable of generating formaldehyde, are effective in processing cellulose containing fibrous materials to impart thereto flame resistance.

The N-methylolated phosphorus compounds having a methylene ether bond, used in the process disclosed in Japanese Pat. No. 691,726, emit a formaldehyde odor and tend to generate formaldehyde easily in the process for flameproofing cellulose containing fibrous materials, thus producing an undesirable working environments.

An object of the present invention is to provide a novel method for reducing the formaldehyde odor associated with the flameproofing of cellulosic containing materials. It is a further object of the present invention to impart to such materials flame resistance coupled with excellent fastness to washing and crease resistance.

Another object of the present invention is to provide novel compounds to enable the above objects.

wherein R<sub>1</sub> to R<sub>4</sub> are the same or different alkyl, alkenyl or alkoxyalkyl groups which may be substituted by one or more chlorine or bromine atoms, and X is a residue of a nitrogen containing compound capable of forming, when reacted with formaldehyde, a dimethylol compound.

**DETAILED DESCRIPTION OF THE INVENTION**

10 The groups R<sub>1</sub> to R<sub>4</sub> in the phosphorus compounds of formula (I) are of 10 or less carbon atoms and preferably of 4 or less carbon atoms. Of these, those phosphorus compounds (I) wherein R<sub>1</sub> to R<sub>4</sub> are alkyl or halogenalkyl groups are preferred, of the alkyl groups methyl group is preferred and of the halogenalkyl groups the chloroethyl group is preferred.

The nitrogen containing compounds capable of forming a dimethylol compound when used as one of the reactants in the preparation of the phosphorus compounds (I), include for example, dialkylureas, cyclic alkyleneureas such as ethyleneurea, and propyleneurea, cyclic alkyleneurea derivatives such as dihydroxyethyleneurea, 5-hydroxypropyleneurea and dialkoxyethyleneurea, urones, triazones, and 4-hydroxy-5, 5-dimethylhexahydroxypyrimidin-2-one and its alkoxy derivatives. Of these ethyleneurea, propyleneurea and N, N'-dimethylurea are preferred.

20 25 30 Although not limited to the following, the preparation of the phosphorus compounds (I) used in accordance with the method of the present invention may conveniently be made by one of the following methods:

35 The first method is a process wherein a dimethylolated nitrogen containing compound is condensed with, for example, 3-dimethylphosphonopropionamide with dehydration, in the presence of an acid catalyst such as p-toluenesulfonic acid. The reaction may be represented as follows:

40



**SUMMARY OF THE INVENTION**

The above enumerated problems are overcome by with the present invention wherein cellulose containing fibrous materials are subjected to flame proofing treatment with a phosphorus compound bearing methylene ether bonds and a residue of a nitrogen containing compound capable of forming a dimethylol compound. These compounds contain no N-methylol groups, and are represented by the following general formula:

50

55

In another process a dimethylolated nitrogen containing compound and monomethylol acrylamide are condensed with water removal in the presence of an acid catalyst to form a divinyl compound bearing methylene ether bonds. The divinyl compound is then reacted with a phosphorous acid ester in the presence of a basic catalyst such as sodium methoxide. The reactions are depicted in the following operation (2).



The phosphorus compounds (I) used in the method of the present invention are characterized by the presence of methylene ether bonds and by the a residue of a nitrogen containing compound capable of forming a dimethylol compound.

It is theorized that when cellulose containing fibrous materials are treated with phosphorus compounds of formula (I), the methylene ether bonds split off and simultaneously react with the hydroxy groups of the cellulosic fiber thereby attaching to the cellulosic fibers in the form of the phosphonopropionamidomethyl ether. As a consequence in the method according to the present invention, it is unnecessary to introduce, by a special method like N-methylolation, other reactive functional groups.

The residue of the nitrogen containing compound, produced by the splitting of methylene ether bonds, provides a cross-linking reaction with the cellulosic fiber, so that the treated cloth exhibits not only flame resistance coupled with excellent fastness upon washing, but also greatly enhanced crease resistance. Since the phosphorus compounds (I) do not emit a formaldehyde odor and do not generate of formaldehyde in the course of processing, the working environment is significantly improved.

The reaction catalysts used to react the cellulose containing materials with the phosphorus compounds of formula (I) used in are those catalysts conventional in the curing of amino resins, for example ammonium chloride, orthophosphoric acid, magnesium chloride, zinc nitrate or zinc borofluoride.

The concentration in the processing solution of the phosphorus compound (I) used, for wetting the cellulosic fibrous materials may be varied in accordance with the desired degree of flame resistance to be imparted, although it will generally be within the range of from 5 to 80 percent by weight, and preferably in the range of from 20 to 50 percent by weight.

The above described processing solutions may be applied to the cellulose containing material, by any of a variety of known methods, such as pressing between rolls, spraying or centrifugation. Likewise, the manner of drying the wetted or impregnated material is conventional and practically any temperature between room temperature and 200°C suffices. With regard to curing conditions, satisfactory results are obtainable by curing at temperatures of the order on from 120° to 200°C for periods of time of from 30 seconds to 10 minutes.

In practicing the method of the present invention, amino resins may simultaneously be applied to the material by inclusion in the treatment bath. Suitable resins include the reaction products of a variety of low molecular amino compounds with formaldehyde and the alkoxylated derivatives thereof. The amino compounds usually used as starting materials for the manufacture of amino resins include, for example, urea, melamine, thiourea, ethyleneurea, guanidine and urone.

When such amino resins are used in combination with the phosphorus compounds (I), however, the working environment deteriorates because of generation of formaldehyde. When the phosphorus compounds (I) are used alone in accordance with the method of the invention, no generation of formaldehyde takes place and therefore the working environment is not adversely affected. Accordingly the application of the phosphorus compounds (I) alone is preferred.

## EXAMPLE 1

Into a reaction flask equipped with means for the removal of reaction and a stirrer are charged 225 g (1.0 mole) monomethyloolated methylethylphosphonopropionamide, 73 g (0.5 mole) freshly prepared dimethylolethyleneurea, 50 g dioxane, 200 g benzene and 1.5 g p-toluenesulfonic acid. The mixture is heated to the boiling point of the benzene, the water formed in the course of the condensation reaction is azeotropically removed and collected in the water separator. Approximately 10 hours after initiating the reaction water formation ceases. The reaction solution is then distilled under reduced pressure to remove the solvent, thus producing 282 g of a clear viscous liquid.

This viscous liquid was found to contain 0.3 percent free formaldehyde, 1.8 percent methylol-type formaldehyde and 19.14 percent methylene ether-type formaldehyde (determined as formaldehyde after decomposition with a dilute aqueous acid solution). The analytic results show that the product is of 89.4 percent purity.

A cotton No. 40 broadcloth was treated in an aqueous solution containing a 30 percent by weight of the product produced above to which solution 0.4 percent ammonium chloride had been added, washed 5 times with a 0.2 percent aqueous detergent aqueous solution and dried. The combustion test with the processed cloth showed incombustibility and the crease resistance of the processed cloth was 287° (original cloth 17.8°).

For comparison, as an example of those phosphorus compounds not bearing a residue of a nitrogen containing compound capable of forming a dimethylol compound, i.e. those phosphorus compounds (I) wherein X is absent, N, N'-oxydimethylenebis(dimethylphosphono) propionamide was synthetized and employed in the same flame proofing process as described above, whereupon the crease resistance was determined to be 180°.

The measurement of the crease resistance was made in accordance with the method of A.A.T.C.C. 88A-1964 T method.

## EXAMPLE 2

Flame resistance tests were conducted with a cotton twill processed with the various urea derivatives as shown in Table 1 below. The composition of each of the respective processing baths as well as the test results before and after washing are also shown in Table 1.

The processing procedure was as follows: The cloth was, after impregnation, picked up (80 percent by weight pick up), dried at 90°C for 4 minutes and cured at 150°C for 4 minutes.

The cured cloth was subjected to 10 minutes of soaping at 40°C in a 0.2 percent by weight detergent (manufactured by Kao Sekken Co., Ltd.; Trade Name ZABU) aqueous solution and then rinsed for 5 minutes with water, this procedure repeated 5 times. The finally dried cloth was used as the test cloth for "after washing."

The flame resistance test was carried out in accordance with Japanese Industrial Standards (JIS)-L-1091 A-1. This test method is also referred to as the 45° microburner method. In this method the test cloth is spread over a 25 × 15 cm frame and set in a combustion test chamber at an angle of 45°. The microburner is ignited, the cloth heated for 1 minute and the flame duration or lasting time (the length of time from the

end of heating to a point where flaming of the test cloth ends) is determined. The microburner is adjusted beforehand to a flame length of 4.5 cm with the tip of the flame in contact with the test cloth. Subsequently, the test cloth is removed from the frame and the carbonized length and area are determined.

or more chlorine or bromine atoms and X is a residue of a urea derivative capable of forming, when reacted with formaldehyde, a dimethylol compound, and drying said flameproofed cellulosic materials

5 2. The method of claim 1 wherein R<sub>1</sub>, R<sub>2</sub>, R<sub>3</sub> and R<sub>4</sub> are alkyl or halogenalkyl groups of 4 or less carbon

Table 1

| R  | X                                                                                 | Processing Bath (% by weight)                                                       |                    |                                |                                | Before Washing |                         |                                     | After Washing            |                         |                                     |                          |   |
|----|-----------------------------------------------------------------------------------|-------------------------------------------------------------------------------------|--------------------|--------------------------------|--------------------------------|----------------|-------------------------|-------------------------------------|--------------------------|-------------------------|-------------------------------------|--------------------------|---|
|    |                                                                                   | Ac-tive agent                                                                       | NH <sub>4</sub> Cl | H <sub>3</sub> PO <sub>4</sub> | M <sub>g</sub> Cl <sub>2</sub> | T-36*          | Carbo-nized length (cm) | Carbo-nized area (cm <sup>2</sup> ) | Flame lasting time (sec) | Carbo-nized length (cm) | Carbo-nized area (cm <sup>2</sup> ) | Flame lasting time (sec) |   |
| 1  |  | 40                                                                                  | —                  | —                              | 2                              | —              | 6.4                     | 20                                  | 0                        | 6.4                     | 23                                  | 0                        |   |
|    |                                                                                   | 30                                                                                  | —                  | 3                              | —                              | —              | 6.4                     | 22                                  | 0                        | 6.4                     | 22                                  | 0                        |   |
|    |                                                                                   | 25                                                                                  | 0.5                | —                              | —                              | —              | 6.6                     | 22                                  | 0                        | 6.8                     | 26                                  | 0                        |   |
| 2  | C <sub>2</sub> H <sub>5</sub>                                                     | 20                                                                                  | —                  | 3                              | —                              | 5              | 6.8                     | 23                                  | 0                        | 7.2                     | 25                                  | 0                        |   |
| 3  | ClC <sub>2</sub> H <sub>4</sub>                                                   | 30                                                                                  | —                  | 3                              | —                              | —              | 6.9                     | 23                                  | 0                        | 6.9                     | 28                                  | 0                        |   |
| 4  | B <sub>2</sub> C <sub>2</sub> H <sub>4</sub>                                      | 30                                                                                  | —                  | 3                              | —                              | —              | 6.9                     | 25                                  | 0                        | 7.2                     | 36                                  | 0                        |   |
| 5  | C <sub>4</sub> H <sub>9</sub> OC <sub>2</sub> H <sub>4</sub>                      | 35                                                                                  | —                  | 3                              | —                              | —              | 7.0                     | 23                                  | 0                        | 7.8                     | 42                                  | 0                        |   |
| 6  | CH <sub>3</sub>                                                                   |    | 30                 | 0.5                            | —                              | —              | 5                       | 6.4                                 | 24                       | 0                       | 6.8                                 | 26                       | 0 |
| 7  | "                                                                                 |    | 30                 | 0.5                            | —                              | —              | —                       | 6.5                                 | 22                       | 0                       | 6.8                                 | 28                       | 0 |
| 8  | "                                                                                 |   | 25                 | —                              | —                              | 2              | 5                       | 6.4                                 | 21                       | 0                       | 6.5                                 | 24                       | 0 |
| 9  | "                                                                                 |  | 30                 | —                              | —                              | 2              | —                       | 6.5                                 | 22                       | 0                       | 7.2                                 | 34                       | 0 |
| 10 | "                                                                                 |  | 30                 | —                              | 3                              | —              | 5                       | 6.6                                 | 20                       | 0                       | 7.0                                 | 32                       | 0 |

\*Trade name "Ulamine T-36" for 30% aqueous methoxymethylolmelamine solution manufactured by Mitsui Toatsu Chemical Co., Ltd.

I claim:

1. A method for flameproofing cellulosic materials comprising applying to the cellulosic material an aqueous solution of a phosphorus compound represented by the following general formula:

35 atoms and X is ethyleneurea, propyleneurea or N, N'-dimethylurea.

3. The method of claim 2 wherein R<sub>1</sub>, R<sub>2</sub>, R<sub>3</sub> and R<sub>4</sub> are methyl groups and X is ethyleneurea.



wherein R<sub>1</sub> to R<sub>4</sub> are the same or different alkyl, alkenyl or alkoxyalkyl groups which may be substituted by one

45 4. The method of claim 2 wherein R<sub>1</sub>, R<sub>2</sub>, R<sub>3</sub> and R<sub>4</sub> are chloroethyl groups and X is ethyleneurea.

\* \* \* \* \*